

## UNITED STATES PATENT OFFICE

2,126,744

## ALLOY

Anthony G. de Golyer, New York, N. Y.

No Drawing. Application August 25, 1936,  
Serial No. 97,742

3 Claims. (Cl. 148—32)

The present invention relates to a new and useful alloy and relates particularly to an alloy containing boron, tungsten, vanadium, zirconium and cobalt, which is characterized by being responsive to thermal treatment for the improvement of physical properties.

An object of the present invention is to provide an alloy especially adapted for use as metal cutting tools, the cutting efficiency of which is superior to that of present known high speed steels and other alloys. A further object is to provide an alloy which is free from, or substantially free from carbon and which is readily amenable to thermal treatment, by means of which the hardness, tensile strength, cutting efficiency and other physical properties and characteristics may be accurately controlled over a comparatively wide range.

I have found through experiment that by alloying or otherwise intimately combining boron, tungsten, vanadium, zirconium and cobalt within the range of boron 0.50% to 3%, tungsten 5% to 30%, vanadium 1% to 8%, zirconium 0.25% to 5%, and cobalt substantially the balance, that I obtain metallic compositions which possess in combination materially improved physical properties compared to those of heretofore known alloys or compositions intended for the cutting or working of metals.

Alloys of this invention may be used in the cast condition but approximate maximum values of hardness, resistance to impact and certain other important physical properties can be developed only through thermal treatment, or through mechanical working and subsequent thermal treatment. Bodies of the alloys which have been subjected to such treatment are particularly valuable for use as tools, dies and the like for the cutting or mechanical working of metals.

Numerous metallic compositions have heretofore been proposed as improvement on the generally known 18-4-1 type of tungsten-chromium-vanadium high speed tool steel, and while many such compositions possess greater hardness than such steel, all of them have disadvantages which render them unsuitable for general application as metal cutting or forming tools. Compositions containing principally carbides of tungsten, molybdenum or tantalum bonded with a relatively soft matrix metal have a high degree of hardness, but are extremely brittle. Cast compositions of the types heretofore proposed require the presence of at least 1.50% carbon to qualify as metal cutting tools and, as is well-known, such alloys

are not only brittle, but are so sensitive to various operating conditions as to greatly restrict the scope of usefulness. One of the greatest disadvantages of such heretofore proposed compositions is that none of them are responsive to thermal treatment for regulation of physical properties, and consequently physical properties and characteristics are governed entirely by the chemical composition of the sintered or cast material.

My alloy may be used in the as-cast condition, or it may be forged or otherwise mechanically worked. In either case I prefer to subject the alloy to thermal treatment before using it as a cutting tool or die. Both the cast and forged material are equally amenable to thermal treatment. For example, cast bodies of this alloy may have a hardness of from 50 to 60 on the Rockwell C. scale and by subjecting the material to suitable thermal treatment, such as quenching from a temperature higher than approximately 1000° C., the hardness may be lowered to an approximate range of from 40 to 47 Rockwell C. In this condition the bodies may be ground, shaped or formed, as desired. The alloy may subsequently be submitted to a second thermal treatment, such as heating to a temperature of less than 1000° C. for a period of one hour or more, by which the hardness may be increased to from approximately 60 to 70 Rockwell C. In the latter condition the alloy is especially valuable for the cutting or mechanical working of a large number of metals and alloys, as well as numerous non-metallic materials. An important property of this alloy is that virtually all of the maximum hardness, developed by thermal treatment, is retained when the alloy is subjected to elevated temperatures, e. g. such as are generated in the tip of a tool cutting metal at high speed. Although the alloy has a high degree of hardness and resistance to abrasion by hot metal chips, especially after thermal treatment, it is remarkably resistant to failure from sudden or repeated shock. Therefore, tools made of the present alloy retain an efficient cutting edge for longer periods than other tools.

The more important distinctive and valuable advantages are, apparently, due to the presence of appreciable amounts of boron in the composition, in conjunction with the other essential component elements within the percentages specified herein.

I have found that molybdenum may be used to supplant all or a portion of the tungsten of the present alloy. Likewise, uranium may be used in place of either tungsten or molybdenum.

Specific examples of compositions within the scope of the present invention which I have found well adapted for metal cutting tools, dies and the like are the following: boron 1.20%, tungsten 5 14%, vanadium 2.75%, zirconium 1.25%, cobalt balance; boron 2.10%, tungsten 19.50%, vanadium 4%, zirconium 0.80%, cobalt balance; boron 1.65%, molybdenum 13%, vanadium 3.5%, zirconium 3.75%, cobalt balance; boron 1.70%. 10 tungsten 5%; molybdenum 10%, vanadium 5%, zirconium 4.60%, cobalt balance; boron 1.10%, molybdenum 12%, vanadium 6%, zirconium 1.75%, cobalt balance.

An objective of the present invention is to provide alloys having high hardness, high resistance to shock and impact, advantageous cutting properties for metal, etc., which are free or substantially free from carbon, and thus eliminate all of the serious disadvantages associated with carbon containing non-ferrous alloys or compositions intended for metal cutting tools. Although I prefer to have the alloys of this invention entirely free from carbon, in many instances I have found carbon present in the nature of an impurity incidental to manufacture. It is important to restrict the amount of carbon so present to a maximum of about 0.15%, as I have found that the presence of higher percentages of this element make the alloy extremely brittle and 20 subject to failure during cutting operations, and, greatly retards or entirely prevents the desired and necessary reactions during thermal treatment. Furthermore, the presence of appreciable amounts of carbon decreases the red hardness 25 of the alloy, i. e. hardness at temperatures of approximately 550° C. and higher.

By reason of the fact that the elements forming the essential components of the alloy of the present invention invariably are contaminated 40 with other elements when produced in commercial quantities, the alloys of my invention usually contain insignificant amounts of one or more elements in the nature of impurities incidental to manufacture. Because of the fact that the maximum values of physical properties of the present 45 alloy can be developed only through thermal treatment, it is essential that the amount of such incidental impurities present be limited to percentages which will not be effective in retarding, or entirely preventing the necessary physical 50 reactions during thermal treatment. Further, the percentages of such impurities should also be restricted to amounts which will not be effective on the physical properties or characteristics of the alloy either before or after thermal treatment.

I have found that the most harmful impurities 60 commonly present, in addition to carbon, are silicon and aluminum. The presence of either of these elements in amounts greater than approximately 1% renders the alloy of the present invention entirely unsuitable for thermal treatment by means of which the hardness, tensile strength and impact resistance and other prop-

erties may be accurately controlled. One of the chief disadvantages of silicon and aluminum is that these elements apparently form chemical compounds with one or more of the essential components of the present alloy, and such compounds are not only hard, brittle and lacking in impact resistance, but are virtually insoluble in the solid composition during thermal treatment. It will be apparent, therefore, that the presence of effective amounts of impurities, such as carbon, silicon and aluminum, materially change the character of the alloy through rendering it not amenable to thermal treatment. 10

My investigations indicate that the preferred structure of a body of the present alloy is produced only by means of thermal treatment, and that this comprises at least two principal constituents: one, a relatively hard intermetallic compound of boron with one or more of the other essential components; and, second, a solid solution of two or more of the essential components which has a lower degree of hardness and functions as a matrix. In some instances the structure will contain a third constituent in the nature of an eutectoid. The ratio of the constituents 20 and the ratio of particle size in any particular body of the alloy may be accurately controlled and fixed over a wide range by means of thermal treatment, or mechanical working and subsequent thermal treatment. 25

By reason of the combined advantageous physical properties possessed by the alloy of the present invention, tools and other articles composed of this alloy may be operated efficiently and economically under conditions which are impossible or uneconomical with tools or articles composed of heretofore known alloys or metallic compositions. 30

By the term "the balance substantially cobalt" in the foregoing and in the following claims, I 40 intend that the alloy of the present invention comprises boron, vanadium, zirconium, and metal of the group tungsten, molybdenum and uranium, within the percentage limits specified, with the remainder cobalt except for ineffective 45 amounts of impurities which may be present incidental to manufacture, as hereinbefore explained.

I claim:

1. A precipitation hardened alloy containing 50 boron 0.50% to 3%, metal from the group tungsten, molybdenum and uranium 5% to 30%, vanadium 1% to 8%, zirconium 0.25% to 5%, the balance cobalt.

2. A precipitation hardened alloy containing 55 boron 0.50% to 3%, tungsten 5% to 30%, vanadium 1% to 8%, zirconium 0.25% to 5%, the balance cobalt.

3. A precipitation hardened alloy containing 60 boron 0.50% to 3%, molybdenum 5% to 30%, vanadium 1% to 8%, zirconium 0.25% to 5%, the balance cobalt.

ANTHONY G. DE GOLYER.